

## UNITED STATES PATENT OFFICE

2,093,738

SENSITIZED BLUE PRINT PAPER AND  
COATING THEREFORAlger P. Reynolds, North Beverly, Mass., assignor  
to Spaulding-Moss Company, Boston, Mass., a  
corporation of MassachusettsNo Drawing. Application February 25, 1936,  
Serial No. 65,661

## 10 Claims.

(Cl. 95—7)

The present invention relates to the art of making "blue prints" by coating a suitable base (which base for the sake of convenience is hereinafter referred to as "paper", but which expression is intended to cover any suitable base which may be used, such as paper, cloth, etc.) with a solution which is sensitive to light so that when the sensitized paper is subsequently exposed to light and then subjected to a suitable developing bath a permanent blue color is obtained wherever the light reached the sensitized paper during exposure.

The primary object of my invention is to provide a more highly sensitive coating for blue print paper which requires exposure to light a shorter period of time during printing, thereby providing a faster paper.

Another object is to provide such a coating which results in a deeper blue background in the exposed areas in the final print.

A further object is to eliminate fogging of the white unexposed surfaces or lines in the final print.

Another object is to provide such an improved sensitized paper which may be kept for longer periods of time in sensitized condition without deterioration prior to exposure to light.

A further object is to provide a coating solution which may be applied to the paper at room temperature, i. e., without heating the solution during coating.

A further object is to provide a coating solution which when applied to the paper causes the paper size to swell or expand thereby permitting more of the coating to be adsorbed by the paper and causing more of the solution to be held thereon.

Other objects are to provide an improved blue print paper coating, and an improved coating solution.

In the prior art it has long been the established practice to sensitize the paper with a coating solution having as its essential elements a water solution of a light-sensitive iron salt in the ferric state, such as ferric ammonium oxalate, and a suitable ferricyanide, such as potassium ferricyanide. When the coated paper has been dried it is fully sensitized and ready for use and is known commercially as "blue print" paper.

In use, an opaque diagram upon transparent or translucent paper (or other suitable medium) is transposed over the sensitized surface of the blue print paper and is then exposed to light for a period of time sufficient to insure reduction of the light-sensitive ferric salt to a ferrous salt. Upon washing the exposed paper with water the ferrous salt combines with the ferricyanide to form an insoluble blue compound, and the unexposed and unreduced ferric salt which is found on the blue print paper beneath the opaque lines

of the diagram is dissolved out of the blueprint paper leaving a white diagram upon a blue background. After being washed with water the exposed paper is commonly washed in a bath containing an oxidizing agent, such as potassium bichromate, thereby bringing out in full the blue background and the paper is then again washed with water and subsequently dried.

Either partial or complete substitution of a ferrocyanide for the ferricyanide in the above-referred to prior art coating bath has been suggested to thereby obtain a faster printing paper which gives sharper white lines upon a deeper blue background. These suggestions will be found in the British patent to Holden No. 418,369 of 1934. In the only suggestions of the use of ferrocyanide found in the prior art, it has been stated that the entire coating solution, i. e., water, light-sensitive ferric salt and ferrocyanide (and ferricyanide, if the latter is also used) must not be acid, and this coating solution as a whole has been made either neutral or alkaline by the use in the solution of suitable combinations of borax, ammonia, sodium hydroxide or potassium oxalate, and the use of these chemicals has been understood by the art to be "buffering" the coating solution to neutral or above, i. e., neutral or alkaline.

When an alkali metal ferrocyanide, such as potassium, sodium or ammonium ferrocyanide, is added to a water solution of a light-sensitive ferric salt, such as ferric ammonium oxalate, a blue substance is formed before exposure to light and after exposure and washing a paper coated with such a coating solution retains a considerable amount of the blue substance upon the unexposed areas, so that these unexposed areas are fogged with blue rather than remaining a clear white. Thus if a ferrocyanide is to be used in a coating solution something must be present which prevents the retention of this blue substance upon the unexposed areas thus permitting it to be washed completely off after printing, leaving clear whites. The art has believed that the incorporation of any suitable "buffer" in this ferrocyanide coating solution to thereby make the solution as a whole neutral or alkaline would prevent this fogging of the whites.

I have found, however, that a much better ferrocyanide coating solution is obtained when the coating solution as whole is acid and not when it is "buffered" to neutral or alkaline, and I have discovered that when one or more of a certain class of chemicals, which I define as alkaline hydrolyzable alkali metal compounds are embodied in the water solution of a light-sensitive ferric salt and an alkali metal ferrocyanide in such quantities that this coating solution as a whole is acid, i. e., with a pH value below 7, not only is this fogging of the whites entirely elimi-

nated but also the paper coated therewith prints considerably faster, with sharper white lines upon a deeper blue background, is easier to keep in sensitized condition, may be coated without heating the coating solution above room temperature, and may be coated so that greater quantities of the solution are more readily and more thoroughly adsorbed by the surface of the paper than by the use of any neutral or alkaline ferrocyanide containing coating solution suggested by the prior art.

By the term "alkali metal" in this specification and the annexed claims, I intend to include only potassium, sodium, cesium, rubidium, lithium, and ammonia, which latter substance although it is not, strictly speaking, a metal, is commonly classed in the alkali metal group. By "alkaline hydrolyzable" compounds or salts wherever said term is used in this specification and the annexed claims, I intend to include only water soluble salts or compounds, the water solutions of which have a pH value of greater than 7.

Thus the class of chemicals referred to as alkaline hydrolyzable alkali metal compounds includes chemicals such as trisodium phosphate, disodium phosphate, trisodium arsenate, disodium arsenate, trisodium citrate, tripotassium citrate, ammonium sodium phosphate, sodium borophosphate, sodium glycerophosphate, magnesium ammonium citrate, sodium pyrophosphate, sodium metasilicate, sodium sesquisilicate, sodium carbonate, sodium bicarbonate, sodium sesquicarbonate, potassium chromate, potassium tartrate, potassium borotartrate, sodium tetraborate, potassium oxalate, sodium hydroxide, potassium hydroxide and ammonium hydroxide. Other chemicals falling within this class will be apparent to those skilled in the art. It will be noted that ammonium sodium phosphate, sodium borophosphate, sodium glycerophosphate, magnesium ammonium citrate, potassium borotartrate, sodium sesquicarbonate and sodium sesquisilicate of the above examples are so called "complex" alkali metal compounds which hydrolyze alkaline. By the term "alkali metal compounds" I intend to include "complex" compounds, so called, in which one or more alkali metals are present and whether or not such compounds contain in addition a metal other than an alkali metal.

Most of these alkaline hydrolyzable alkali metal compounds when incorporated either separately or in combination with each other in a water solution of a light-sensitive iron salt in the ferric state, such as ferric ammonium oxalate, and a suitable ferrocyanide, such as potassium ferrocyanide (with or without a ferricyanide), produce a coating solution which has a pH value below 7 and is therefore acid. However, the above-mentioned hydroxides and a very few of the above-mentioned salts, such as sodium tetraborate or potassium oxalate, when used together in certain proportions and incorporated in the water solution of the light-sensitive iron salt in the ferric state and the ferrocyanide (with or without a ferricyanide), produce a coating solution which is neutral or alkaline as a whole. For instance, the coating solution in the example given at page 2 of the Holden British patent has a pH value of 7.2. In accordance with my invention the pH value of such a coating solution must be reduced below 7, and this may be done by adding suitable proportions of weak inorganic acids, such as pyrophosphoric, orthophosphoric, boric, silicic, carbonic, or arsenic, or suitable proportions of certain organic acids, such as oxalic, cit-

ric, tartaric, or malonic, or suitable proportions of a salt which hydrolyzes acid and is formed by the reaction between an alkali metal and certain of said weak inorganic acids, such as phosphoric, or certain of said organic acids, such as oxalic, citric, or tartaric. Examples of such salts are monopotassium orthophosphate, monosodium orthophosphate, sodium binoxalate, sodium bitartrate and sodium acid citrate. The addition of suitable proportions of such acids or such salts which hydrolyze acid will make the coating solution as a whole acid without at the same time resulting in the above-mentioned fogging of the whites.

Of the above class which I have defined as alkaline hydrolyzable alkali metal compounds, I prefer to use a subclass comprising alkaline hydrolyzable salts of an alkali metal and a weak acid. By the term "salts of an alkali metal and a weak acid" I intend to include so-called "complex" salts in which one or more alkali metals and one or more weak acid radicals are present, and such "complex" salts may contain in addition a metal other than an alkali metal or acid radicals other than weak acid radicals. An example of such a "complex" alkaline hydrolyzable salt of an alkali metal and a weak acid is magnesium ammonium citrate, and this is such a salt notwithstanding the presence of the non-alkali metal magnesium. By the term "weak acid" in this specification and the annexed claims, I intend to include only acids whose dissociation constants are equal to or less than the dissociation constant of pyrophosphoric acid. For example, hydrochloric, sulphuric and nitric acids would not be "weak acids" for the purpose of this class, since their dissociation constants are greater than that of pyrophosphoric acid. Examples of alkaline hydrolyzable salts of an alkali metal and a weak acid are trisodium phosphate, disodium phosphate, trisodium arsenate, disodium arsenate, trisodium citrate, tripotassium citrate, ammonium sodium phosphate, sodium borophosphate, sodium glycerophosphate, magnesium ammonium citrate, sodium pyrophosphate, sodium metasilicate, sodium sesquisilicate, sodium carbonate, sodium bicarbonate, sodium sesquicarbonate, potassium chromate, potassium tartrate, potassium borotartrate, sodium tetraborate, and potassium oxalate. Other members of this class will be apparent to persons skilled in the art.

An example of a suitable coating solution using trisodium orthophosphate, a member of this class, is as follows:

200 grams of ferric ammonium oxalate and 30 grams of trisodium orthophosphate dissolved in 500 cc. of water, and to this solution add: 30 grams of potassium ferrocyanide and 25 grams of potassium ferricyanide dissolved in 60 500 cc. of water.

This solution is of a deep blue color and has a pH value of 6.11. If the ferricyanide is replaced in whole or in part by ferrocyanide in the above example, the amount of trisodium orthophosphate should ordinarily be increased. It will be apparent to persons skilled in the art that if an alkali metal ion is present in a coating solution containing a light-sensitive ferric salt and a ferrocyanide, the incorporation of any weak acid into such a solution to thereby form with the alkali metal an alkali metal salt which hydrolyzes alkaline would be within the scope of this invention as equivalent to the use ab initio of 75

an alkaline hydrolyzable salt of an alkali metal and a weak acid.

Of the above class which I have defined as alkaline hydrolyzable salts of an alkali metal and a weak acid, I prefer to use a further subclass comprising alkaline hydrolyzable salts of an alkali metal and a weak polyvalent acid. By the term "salts of an alkali metal and a weak polyvalent acid" I intend to include any of the so-called "complex" salts in which one or more alkali metals and one or more weak polyvalent acid radicals are present whether or not such salts contain in addition metals other than alkali metals or acid radicals other than weak polyvalent acid radicals. By the term "weak polyvalent acids" I intend to include only polyvalent acids whose dissociation constants are equal to or less than the dissociation constant of pyrophosphoric acid. For example, sulphuric acid is a polyvalent acid, the alkali metal salts of which would not fall within this class, since its dissociation constant is greater than that of pyrophosphoric acid.

All of the alkaline hydrolyzable salts enumerated above as examples of salts of an alkali metal and a weak acid, happen to also be such salts of weak polyvalent acids, and the said chemicals are here again referred to as examples of this subclass. Other members of this class will be apparent to persons skilled in the art. The coating solution of trisodium orthophosphate given above will also serve as an example of a suitable coating solution under this class.

If an alkali metal ion is present in a coating solution containing a light-sensitive ferric salt and a ferrocyanide, the incorporation into such a solution of any weak polyvalent acid to thereby form an alkali metal salt which hydrolyzes alkaline, would be within the scope of this invention as equivalent to the use ab initio of an alkaline hydrolyzable salt of an alkali metal and a weak polyvalent acid.

Of the subclass which I have defined as alkaline hydrolyzable salts of an alkali metal and a weak polyvalent acid, I prefer to use a member of a further subclass comprising alkaline hydrolyzable salts of an alkali metal and a trivalent acid. By the term "salts of an alkali metal and a trivalent acid" I intend to include any of the so-called "complex" salts in which one or more alkali metals and one or more trivalent acid radicals are present whether or not such salts contain in addition metals other than alkali metals or acid radicals other than trivalent acid radicals. Examples of members of this class are trisodium phosphate, disodium phosphate, trisodium arsenate, disodium arsenate, trisodium citrate, tripotassium citrate, ammonium sodium phosphate, sodium borophosphate, sodium glycerophosphate, and magnesium ammonium citrate. Other members of this class will be apparent to persons skilled in the art.

An example of a suitable coating solution using tripotassium citrate, a member of this class, is as follows:

200 grams of ferric ammonium oxalate and 25.5 grams of tripotassium citrate dissolved in 500 cc. of water, and to this solution add: 70 30 grams of potassium ferrocyanide and 25 grams of potassium ferricyanide dissolved in 500 cc. of water.

This solution is of a deep blue color and has a pH value of 5.22. If the ferricyanide is replaced 75 in whole or in part by ferrocyanide in the above

example, the amount of tripotassium citrate should ordinarily be increased. The use of a trivalent acid to form an alkaline hydrolyzable alkali metal salt with alkali metal ions present in the coating solution is within the scope of this 5 invention as equivalent to the use ab initio of an alkaline hydrolyzable salt of an alkali metal and a trivalent acid.

Of the subclass which I have defined as alkaline hydrolyzable salts of an alkali metal and a weak polyvalent acid, I next prefer to use a member of the subclass comprising alkaline hydrolyzable salts of an alkali metal and a weak divalent acid. By the term "salts of an alkali metal and a weak divalent acid" I intend to include any of the so-called "complex" salts in which one or more alkali metals and one or more weak divalent acid radicals are present whether or not such salts contain in addition metals other than alkali metals or acid radicals other than weak divalent acid radicals. By the term "weak divalent acid" I intend to include only divalent acids whose dissociation constants are equal to or less than the dissociation constant of pyrophosphoric acid. For example, sulphuric acid is 25 a divalent acid, the alkali metal salts of which would not fall within this class since its dissociation constant is greater than that of pyrophosphoric acid. Examples of members of this 30 class are, sodium metasilicate, sodium sesquisilicate, sodium carbonate, sodium bicarbonate, sodium sesquicarbonate, potassium chromate, potassium tartrate, potassium borotartrate, sodium tetraborate, and potassium oxalate. Other members of this class will be apparent to persons 35 skilled in this art. An example of a suitable coating solution using sodium metasilicate, a member of this class, is as follows:

200 grams of ferric ammonium oxalate and 40 16.75 grams of sodium metasilicate dissolved in 500 cc. of water, and to this solution add:

30 grams of potassium ferrocyanide and 25 grams of potassium ferricyanide dissolved 45 in 500 cc. of water.

This solution is of a deep blue color and has a pH value of 6.81. If the ferrocyanide is replaced in whole or in part by ferrocyanide in the above example, the amount of sodium metasilicate should ordinarily be increased. The use of a weak divalent acid to form an alkaline hydrolyzable alkali metal salt with alkali metal ions present in the coating solution is within the scope of this invention as equivalent to the use ab 50 initio of an alkaline hydrolyzable salt of an alkali metal and a weak divalent acid.

Of the class which I have defined as alkaline hydrolyzable salts of an alkali metal and a weak polyvalent acid, I most prefer to use the subclass comprising alkaline hydrolyzable alkali metal phosphates, and of these I prefer sodium pyrophosphate. By the term "alkali metal phosphates" I intend to include the so-called "complex" compounds in which one or more alkali 65 metals and one or more phosphate radicals are present whether or not such compounds contain in addition metals other than alkali metals or acid radicals other than phosphate radicals. Examples of so-called "complex" compounds herein included in the term "alkaline hydrolyzable alkali metal phosphates" are sodium borophosphate, sodium glycerophosphate, ammonium sodium phosphate, and magnesium ammonium phosphate. Other members of this class are tri- 75

sodium phosphate, disodium phosphate, and sodium pyrophosphate. Other members of this class will be apparent to persons skilled in this art.

5 A suitable coating solution embodying my preferred embodiment of this class, trisodium orthophosphate, has been given above.

An example of a coating solution using sodium pyrophosphate, a member of this class, is as follows:

10 200 grams of ferric ammonium oxalate and 20.0 grams of sodium pyrophosphate dissolved in 500 cc. of water, and to this solution add:

15 30 grams of potassium ferrocyanide and 25 grams of potassium ferricyanide dissolved in 500 cc. of water.

20 This solution is of a deep blue color and has a pH value of 5.83. If the ferricyanide is replaced in whole or in part by ferrocyanide in the above example, the amount of sodium pyrophosphate should ordinarily be increased.

25 An example of a coating solution using sodium borophosphate, another member of this class, is as follows:

30 200 grams of ferric ammonium oxalate and 24.0 grams of sodium borophosphate dissolved in 500 cc. of water, and to this solution add:

35 30 grams of potassium ferrocyanide and 25 grams of potassium ferricyanide dissolved in 500 cc. of water.

40 This solution is of a deep blue color and has a pH value of 5.61. If the ferricyanide is replaced in whole or in part by ferrocyanide in the above example, the amount of sodium borophosphate should ordinarily be increased.

45 It will be apparent to one skilled in the art that if alkali metal ions are present in a coating solution containing a light-sensitive ferric salt and a ferrocyanide, the incorporation of phosphates or any phosphoric acid into such a solution to thereby form an alkali metal phosphate which hydrolyzes alkaline would be within the scope of this invention as equivalent to use ab initio of an alkali metal phosphate which hydrolyzes 50 alkaline.

55 Of the class which I have defined as alkaline hydrolyzable alkali metal compounds, the subclass which I least prefer to use is the class comprising the alkali metal hydroxides of which class sodium, potassium and ammonium hydroxides are representative members. Other members of this class will be apparent to persons skilled in this art. A suitable coating solution using sodium hydroxide is as follows:

60 200 grams of ferric ammonium oxalate and 3.25 grams of sodium hydroxide dissolved in 500 cc. of water, and to this solution add:

65 30 grams of potassium ferrocyanide and 25 grams of potassium ferricyanide dissolved in 500 cc. of water.

70 This solution is of deep blue color and has a pH value of 6.78.

75 As hereinabove pointed out, these hydroxides if used in sufficient quantities tend to bring the coating solution to neutral or alkaline. A suitable coating solution using monopotassium phosphate (a suitable alkali metal salt which hy-

drolyzes acid as hereinabove stated) in addition to sodium hydroxide is as follows:

200 grams of ferric ammonium oxalate, and 6.0 grams of sodium hydroxide, and 11.0 grams of monopotassium phosphate dissolved in 500 cc. of water, and to this solution add:

30 grams of potassium ferrocyanide and 25 grams of potassium ferricyanide dissolved in 500 cc. of water.

10 This solution is of a deep blue color and has a pH value of 5.88.

15 It will be apparent to persons skilled in this art that it is within the scope of this invention and the annexed claims to first coat the paper with a sizing containing, or to prepare a paper with a sizing containing, one or more alkaline hydrolyzable alkali metal compounds and then to subsequently coat this paper with a solution 20 containing a light-sensitive ferric salt and a ferrocyanide, since the two coatings would combine to form the coating of this invention.

25 In this specification and the annexed claims when I refer to a coating containing alkaline hydrolyzable alkali metal compounds, light sensitive iron salts in the ferric state and ferrocyanides, I intend to include a coating solution containing, a coating containing, and a paper coated with a coating containing the reaction 30 products of said alkali metal compounds, said light-sensitive ferric salts and said ferrocyanides because I do not know whether or not said chemicals retain their original identity after they are brought together in a coating solution 35 or a coating.

40 It will be understood that the use of ferricyanide may be entirely eliminated in any of my coating solutions hereinabove described, and also that the proportions of ferricyanide to ferrocyanide may be varied at will as has been indicated. Generally speaking the more ferricyanide present in relation to the ferrocyanide 45 present, the slower is the printing speed.

45 It will also be understood that more than one of the alkaline hydrolyzable alkali metal compounds may be used in the same coating solution even though these compounds are selected from different subclasses as defined in this 50 specification.

55 It will be further understood that chemicals other than alkali metal compounds which hydrolyze alkaline, light-sensitive ferric salts, ferrocyanides, and ferricyanides may be incorporated in the coating solution or in the coating 60 on the paper without departing from my invention. So long as the water solution of the coating is acid and contains at least one alkaline hydrolyzable alkali metal compound, a light-sensitive ferric salt, and an alkali metal ferrocyanide, it is intended to be within the scope of the annexed claims, even if the coating solution or the coating on the paper contains other chemicals in addition to those specified.

65 Suitable light-sensitive iron salts in the ferric state other than ferric ammonium oxalate, suitable alkali metal ferrocyanides other than potassium ferrocyanide, and suitable ferricyanides other than potassium ferricyanide will be apparent to those skilled in the art.

70 The determination of the alkalinity, neutrality, or acidity of hydrolyzation of the compounds and salts recited in this specification and the determination of the pH values of coating solutions given in this specification has been made 75

by utilizing a potentiometer and a glass electrode, which method is well known to those skilled in the art and which is the only method now known to me by which the pH values of these coating solutions and pH values of hydrolyzation of all of the compounds and salts relating to this invention can be accurately determined. By an acid coating solution I mean one which has a pH value of less than 7 and which value is determined by said method or by one which is equivalently accurate. By an alkaline hydrolyzable compound or salt I mean one the water solution of which has a pH value greater than 7 and which value is accurately determined by said method or its equivalent.

Persons practicing this invention should guard against using appreciable quantities of a salt or compound which is extremely strong in its reducing effect, since such a salt will tend to reduce the light-sensitive iron salt before the paper is exposed to light and thus destroy or deteriorate the light-sensitiveness of the coating. Sodium sulphite is an example of such a salt.

In use the paper is sensitized by coating at least one surface thereof with a coating solution made in accordance with this invention, and it is then dried and ready for use. Such a coated paper is dark blue-green in color as distinguished from the lemon-yellow color of prior art paper. The coating may be effected by brushing, by spraying, by passing the paper through a machine in contact with rollers which dip into a bath of the solution or by any other suitable coating procedure. The diagram is then superimposed upon the sensitized surface of the dry paper, is printed by exposure to light, and the printed or exposed paper is passed through a water bath after which it may be hung up to dry. If desired, before this final drying the paper may be passed through an oxidizing bath, then through another water bath and then dried.

The acidity of the coating solution as a whole increases the speed of reduction of the light-sensitive iron salt and thus an acid coating solution provides a much faster printing paper than a coating solution which is neutral or alkaline.

Paper coated with the acid coating solutions of a light-sensitive ferric salt and ferrocyanide made in accordance with my invention may be kept in sensitized condition without spoilage for much longer periods of time before exposure than the papers of the prior art, and will produce perfectly clear and unfogged whites when subsequently printed. The acidity of my coating solution causes the size in the paper to swell and thus to absorb the coating solution much more readily than neutral or alkaline solutions, and consequently a less concentrated coating solution is required to provide sufficient of the sensitized coating upon the surface of the paper for a satisfactory deep blue background in the final print, whereas in the use of neutral or alkaline solutions it is necessary to use solutions which are highly concentrated and which require heating to keep the chemicals in solution before and during coating.

It is to be understood that my invention is not dependent upon the theories which I have set forth as descriptive of the chemical actions involved nor dependent upon the soundness or accuracy of theoretical statements so advanced, such theories or theoretical statements are merely what I believe to be correct and I intend to claim

everything inherent in my invention which is novel in view of the prior art.

I claim:

1. A sensitized blue print paper coating containing an alkaline hydrolyzable alkali metal compound, a light-sensitive iron salt in the ferric state and an alkali metal ferrocyanide, the proportions of said alkali metal compound to the other ingredients of the coating being such that a water solution of said coating has a pH value of less than 7 but not sufficiently low to permit the formation of an insoluble blue compound prior to exposure to light.

2. A sensitized blue print paper coating containing an alkaline hydrolyzable salt of an alkali metal and a weak acid, a light-sensitive iron salt in the ferric state and an alkali metal ferrocyanide, the proportions of said alkaline hydrolyzable salt to the other ingredients of the coating being such that a water solution of said coating has a pH value of less than 7 but not sufficiently low to permit the formation of an insoluble blue compound prior to exposure to light.

3. A sensitized blue print paper coating containing an alkaline hydrolyzable salt of an alkali metal and a weak polyvalent acid, a light-sensitive iron salt in the ferric state and an alkali metal ferrocyanide, the proportions of said alkaline hydrolyzable salt to the other ingredients of the coating being such that a water solution of said coating has a pH value of less than 7 but not sufficiently low to permit the formation of an insoluble blue compound prior to exposure to light.

4. A sensitized blue print paper coating containing an alkaline hydrolyzable salt of an alkali metal and a weak divalent acid, a light-sensitive iron salt in the ferric state and an alkali metal ferrocyanide, the proportions of said alkaline hydrolyzable salt to the other ingredients of the coating being such that a water solution of said coating has a pH value of less than 7 but not sufficiently low to permit the formation of an insoluble blue compound prior to exposure to light.

5. A sensitized blue print paper coating containing an alkaline hydrolyzable salt of an alkali metal and a weak trivalent acid, a light-sensitive iron salt in the ferric state and an alkali metal ferrocyanide, the proportions of said alkaline hydrolyzable salt to the other ingredients of the coating being such that a water solution of said coating has a pH value of less than 7 but not sufficiently low to permit the formation of an insoluble blue compound prior to exposure to light.

6. A sensitized blue print paper coating containing an alkaline hydrolyzable alkali metal phosphate, a light-sensitive iron salt in the ferric state and an alkali metal ferrocyanide, the proportions of said alkali metal phosphate to the other ingredients of the coating being such that a water solution of said coating has a pH value of less than 7 but not sufficiently low to permit the formation of an insoluble blue compound prior to exposure to light.

7. A sensitized blue print paper coating containing an alkali metal hydroxide, a light-sensitive iron salt in the ferric state and an alkali metal ferrocyanide, the proportions of said alkali metal hydroxide to the other ingredients of the coating being such that a water solution of said coating has a pH value of less than 7 but not sufficiently low to permit the formation of an insoluble blue compound prior to exposure to light.

8. A sensitized blue print paper coating containing sodium metasilicate, a light-sensitive iron salt in the ferric state and an alkali metal ferrocyanide, the proportions of said sodium metasilicate to the other ingredients of the coating being such that a water solution of said coating has a pH value of less than 7 but not sufficiently low to permit the formation of an insoluble blue compound prior to exposure to light.
10. 9. A sensitized blue print paper coating containing sodium pyrophosphate, a light-sensitive iron salt in the ferric state and an alkali metal ferrocyanide, the proportions of said sodium pyrophosphate to the other ingredients of the coat-
- ing being such that a water solution of said coating has a pH value of less than 7 but not sufficiently low to permit the formation of an insoluble blue compound prior to exposure to light. 5
10. A sensitized blue print paper coating containing sodium hydroxide, a light-sensitive iron salt in the ferric state and an alkali metal ferrocyanide, the proportions of said sodium hydroxide to the other ingredients of the coating being such that a water solution of said coating has a pH value of less than 7 but not sufficiently low to permit the formation of an insoluble blue compound prior to exposure to light. 10

ALGER P. REYNOLDS.